# EUROPEAN PATENT SPECIFICATION

(11) **EP 1 031 415 B1**
(45) Date of publication and mention of the grant of the patent: **24.05.2006**
(21) Application number: 99200528.0
(22) Date of filing: 23.02.1999
(51) Int. Cl.: B41C 1/10

(54) **Dry method for preparing a thermal lithographic printing plate precursor**
Trockenverfahren zur Herstellung von einer thermischen Flachdruckformen-Vorstufe
Procédé à sec pour la préparation de précurseur de plaque d'impression lithographique thermique

(43) Date of publication of application: 30.08.2000
(73) Proprietor: AGFA-GEVAERT, 2640 Mortsel (BE)
(72) Inventor: Vermeersch, Joan c/o Agfa-Gevaert N.V., 2640 Mortsel (BE); Leenders, Luc c/o Agfa-Gevaert N.V., 2640 Mortsel (BE); Meisters, Augustin c/o Agfa-Gevaert N.V., 2640 Mortsel (BE)

(56) References cited:
- EP-A- 0 099 264
- EP-A- 0 786 337
- GB-A- 1 157 918
- US-A- 5 683 848
- A.S.DIAMOND: "HANDBOOK OF IMAGING MATERIALS" , MARCEL DEKKER , NEW YORK XP002111081 * page 165, paragraph 4.2.1 - page 166 * * page 168, paragraph 4.2.2 *

## Description

### FIELD OF THE INVENTION

The present invention relates to a method for making a heat-mode lithographic printing plate precursor and a lithographic printing master in computer-to-plate and computer-to-press procedures.

### BACKGROUND OF THE INVENTION

Rotary printing presses use a so-called master such as a printing plate which is mounted on a cylinder of the printing press. The master carries an image which is defined by the ink accepting areas of the printing surface and a print is obtained by applying ink to said surface and then transferring the ink from the master onto a substrate, which is typically a paper substrate. In conventional lithographic printing, ink as well as an aqueous fountain solution are fed to the printing surface of the master, which is referred to herein as lithographic surface and consists of oleophilic (or hydrophobic, i.e. ink accepting, water repelling) areas as well as hydrophilic (or oleophobic, i.e. water accepting, ink repelling) areas.

Printing masters are generally obtained by the so-called computer-to-film method wherein various pre-press steps such as typeface selection, scanning, colour separation, screening, trapping, layout and imposition are accomplished digitally and each colour selection is transferred to graphic arts film using an image-setter. After processing, the film can be used as a mask for the exposure of an imaging material called plate precursor and after plate processing, a printing plate is obtained which can be used as a master.

In recent years the so-called computer-to-plate method has gained a lot of interest. This method, also called direct-to-plate method, bypasses the creation of film because the digital document is transferred directly to a plate precursor by means of a so-called plate-setter. In the field of such computer-to-plate methods the following improvements are being studied presently :
(i) On-press imaging. A special type of a computer-to-plate process, involves the exposure of a plate precursor while being mounted on a plate cylinder of a printing press by means of an image-setter that is integrated in the press. This method may be called 'computer-to-press' and printing presses with an integrated image-setter are sometimes called digital presses. A review of digital presses is given in the Proceedings of the Imaging Science & Technology's 1997 International Conference on Digital Printing Technologies (Non-Impact Printing 13). Computer-to-press methods have been described in e.g. **EP-A 770 495, EP-A 770 496, WO 94001280, EP-A 580 394** and **EP-A 774 364**. The best known imaging methods are based on ablation. A problem associated with ablative plates is the generation of debris which is difficult to remove and may disturb the printing process or may contaminate the exposure optics of the integrated image-setter. Other methods require processing with chemicals which may damage the electronics and other devices of the press.
(ii) On-press coating. Whereas a plate precursor normally consists of a sheet-like support and one or more functional coatings, computer-to-press methods have been described wherein a composition, which is capable to form a lithographic surface upon image-wise exposure and optional processing, is provided directly on the surface of a plate cylinder of the press. **EP-A 101 266** describes the coating of a hydrophobic layer directly on the hydrophilic surface of a plate cylinder. After removal of the non-printing areas by ablation, a master is obtained. However, ablation should be avoided in computer-to-press methods, as discussed above. **US-P 5,713,287** describes a computer-to-press method wherein a so-called switchable polymer such as tetrahydro-pyranyl methylmethacrylate is applied directly on the surface of a plate cylinder. The switchable polymer is converted from a first water-sensitive property to an opposite water-sensitive property by imagewise exposure. The latter method requires a curing step and the polymers are quite expensive because they are thermally unstable and therefore difficult to synthesise. **EP-A 802 457** describes a hybrid method wherein a functional coating is provided on a plate support that is mounted on a cylinder of a printing press. This method also needs processing. A major problem associated with known on-press coating methods is the need for a wet-coating device which needs to be integrated in the press.
(iii) Elimination of chemical processing. The development of functional coatings which require no processing or may be processed with plain water is another major trend in plate making. **WO 90002044, WO 91008108** and **EP-A 580 394** disclose such plates, which are, however, all ablative plates. In addition, these methods require typically multi-layer materials, which makes them less suitable for on-press coating. A non-ablative plate which can be processed with plain water is described in e.g. **EP-A 770 497** and **EP-A 773 112**. Such plates also allow on-press processing, either by wiping the exposed plate with water while being mounted on the press or by the fountain solution during the first runs of the printing job.
(iv) Thermal imaging. Most of the computer-to-press methods referred to above use so-called thermal materials, i.e. plate precursors or on-press coatable compositions which comprise a compound that converts absorbed light into heat. The heat which is generated on image-wise exposure triggers a (physico-)chemical process, such as ablation, polymerisation, insolubilisation by cross-linking of a polymer, decomposition, or particle coagulation of a thermoplastic polymer latex. This heat-mode process then results in a lithographic surface consisting of ink accepting and ink repelling areas.
   **GB-A 1157918** describes a method comprising the steps of coating a surface with a dry powder toner, focusing a laser beam onto the surface to form images and removing the excess toner from the surface. The surface can be a a hydrophilic printing plate and the toner can be oleophilic, for example an electrofax toner. By wetting the plate in water and then applying an oil based ink, a printing plate is provided for lithographic printing.

**EP-A- 786 337** discloses a process for imaging a printing plate, wherein the printing plate is charged over the whole surface and over the whole surface is covered with toner particles, which are charged oppositely. Thereon is the layer, formed by the particles imagewise fixed or imagewise ablated by infrared exposure on the surface of the printing plate. Thereafter the parts which are not fixed are removed and optionally the non-ablated areas are fixed by heating over the whole surface of the plate. This process requires a cumbersome development.

A problem associated with most thermal materials disclosed in the prior art is that these materials are suitable for exposure with either an internal drum image-setter (i.e. typically a high-power short-time exposure) or an external drum image-setter (i.e. relatively low-power long-time exposure). Providing a universal material that can be exposed with satisfactory results on both these types of laser devices known in the art is a requirement difficult to fulfil.

### OBJECTS OF THE INVENTION

It is an object of the present invention to provide a cost effective method for preparing a material which is suitable for making a printing master for conventional lithographic printing by using computer-to-plate, computer-to-press or on-press coating methods and which requires no processing or can be processed with plain water. It is another object of the present invention to provide a method for making a universal material which can be exposed with internal as well as external drum image-setters.

Further advantages of the present invention will become apparent from the following description.

### SUMMARY OF THE INVENTION

According to the present invention there is provided a method for making a negative working non-ablative imaging material, suitable for making a lithographic printing plate, comprising the steps of applying a dry powder containing at least a compound capable of converting light into heat and an organic compound on a surface of a non-electrically charged metal support, characterized in that the amount of organic compound in said powder ranges from 51 to 95% by weight.

### DETAILED DESCRIPTION OF THE INVENTION

Said organic compound is present in said powder in an amount of at least 51%. Said organic compound is preferably a thermoplastic polymer particle, more preferably with a diameter between 0.02 µm and 10 µm, most preferably between 0.050 µm and 2 µm. Preferred thermoplastic polymers are novolac, polystyrene or a polyacrylate, used alone or mixed with one or two of the other components. Preferably said thermoplastic polymer particles contain a reactive compound inside or outside these particles. Particles containing reactive compounds inside the particles are prepared according to the well known technique of preparing microcapsules or by adding the reactive compound in a water immiscible solvent to the particles dispersed in water. Particles containig reactive compounds outside the particles are prepared according to the well known technique of loading latices as described in **EP-A- 483 416**. Reactive compounds are compounds which can cause cross-linking. Preferred reactive compounds are melamine resins, urethanes, phenol-formaldehyde resins and epoxy compounds.

The compound which is capable of converting light into heat is preferably an organic dye or pigment, carbon black, graphite, metal carbides, borides, nitrides, carbonitrides, or oxides.

The materials made by the method of the present invention are preferably sensitive to near infrared light. Accordingly, the compound capable of converting light into heat is preferably a near infrared light absorbing compound such as carbon or an infrared dye. It is also possible to use dry, finely divided polymer particles consisting of e.g. a polypyrrole or polyaniline-based polymer. The infrared dyes listed in Table 1 are highly preferred.

The amount of the compound capable of converting light into heat is in the range of 5 to 49% by weight, more preferably between 10 to 49% by weight of the dry powder.

The compound capable of converting light into heat can also be incorporated in or adsorbed to or mixed with the polymeric particles or is heterogeneously mixed with said organic compound.

The materials made by the method of the present invention require no processing or can be processed with plain water. Since it is a dry coating method, the method of the present invention is very suitable for computer-to-press applications and on-press coating procedures.

The imaging mechanism of the materials that are made according to the present invention is not known, but may rely on a thermal interaction between the light absorbing compound and the metal support.

The features of the present invention, as specified in the claims, shall be understood as indicated hereafter. The word "image" is used herein in the context of lithographic printing, i.e. "a pattern consisting of oleophilic and hydrophilic areas". The material that is made according to the present invention is negative working, which means that the areas, which are exposed to light, are rendered oleophilic and thus ink accepting due to said exposure. In the context of the present invention, the feature "negative working" may be considered as an equivalent of the feature "non-ablative", since in ablative materials the functional layers are completely removed from the underlying (hydrophilic) metal support upon imagewise exposure so as to obtain a positive image (exposed areas are hydrophilic, ink repelling). Analysis of the exposed areas of the material made according to the method of the present invention indeed showed that the layer or stack of layers is not removed upon image-wise exposure but is converted into a hydrophobic surface on the metal support. The unexposed areas are hydrophilic or become hydrophilic after processing with plain water.

The dry powder used in the present invention may further comprise non-reactive compounds, i.e. inert components such as e.g. a matting agent or a filler. The word "inert" shall not be understood in the meaning of "non-functional", since these inert compounds may be added to the powder to adjust certain physical properties, such as e.g. surface roughness and friction coefficient of the applied layer or the rheological properties of the powder. The word "inert" shall rather be understood as meaning "not essential for the imaging process", though some inert compounds may have a (minor) influence on the speed and image quality of the material.

The method of the present invention may be used to apply a stack of layers on a metal support but a single layer is preferred. The compound capable of converting light into heat may be present in all the layers of said stack or may be localised in just a single layer of said stack. In a method according to the latter embodiment the layer comprising the compound capable of converting light into heat is preferably applied directly on the metal support. The layer comprising the compound capable of converting light into heat is preferably very thin, i.e. having a dry layer thickness below 2 µm, preferably not higher than 1 µm.

The support used in the present invention is a non-electrically charged metal support. Preferred examples of said metal support are steel, especially polished stainless steel, and aluminium. Phosphor bronze (an alloy comprising >90 wt.% of copper, <10 wt.% of tin and small amounts of phosphor) can also be used. The aluminium support is preferably an electrochemically grained and anodised aluminium support. Most preferably said aluminium support is grained in nitric acid, yielding imaging elements with a higher sensitivity. The anodised aluminium support may be treated to improve the hydrophilic properties of its surface. For example, the aluminium support may be silicated by treating its surface with sodium silicate solution at elevated temperature, e.g. 95°C.
Alternatively, a phosphate treatment may be applied which involves treating the aluminium oxide surface with a phosphate solution that may further contain an inorganic fluoride. Further, the aluminium oxide surface may be rinsed with a citric acid or citrate solution. This treatment may be carried out at room temperature or can be carried out at a slightly elevated temperature of about 30 to 50°C. A further treatment may involve rinsing the aluminium oxide surface with a bicarbonate solution. Still further, the aluminium oxide surface may be treated with poly(vinyl phosphonic acid), poly(vinyl methylphosphonic acid), phosphoric acid esters of poly(vinyl alcohol), poly(vinyl sulphonic acid), poly(vinyl benzenesulphonic acid), sulphuric acid esters of poly(vinyl alcohol), and acetals of poly(vinyl alcohols) formed by reaction with a sulphonated aliphatic aldehyde. It is evident that one or more of these post treatments may be carried out alone or in combination.

A highly preferred material made according to the present invention comprises a non-electrically charged anodised aluminium support and provided directly thereon a single recording layer which consists essentially of a compound capable of converting light into heat and thermoplastic polymer particles. On top of said recording layer there may be provided a top layer for protecting the recording layer against moisture, chemicals, oxygen, mechanical impact, etc.

According to the present invention, a non-electrically charged metal support can be applied with a dry powder by rubbing in the surface of said support with said dry powder. Alternative dry coating methods can also be used, e.g. sputter-coating of the powder on the metal support.

The method of the present invention can be used in computer-to-plate (off-press exposure) or computer-to-press (on-press exposure) procedures. The method may also involve on-press coating, i.e. applying a dry powder according to the present invention directly on the non-electrically charged metal surface of a cylinder of a rotary printing press. Said on-press coating can also be performed indirectly by applying the dry powder on a metal support which is mounted on a cylinder of a rotary printing press. In still another method according to the present invention, said composition can be applied on a metal sleeve which, after image-wise exposure and optional processing, is then transferred to a cylinder of a rotary printing press.

The dry powder may also be applied on the non-electrically charged metal support by contacting the surface of said support with another material, which carries a dry layer containing an organic compound and a compound capable of transferring light into heat which are then transferred to the metal support. The method of this embodiment can be automated easily, e.g. by incorporating a supply roll of such a transfer material, such as a ribbon impregnated with the dry powder in a print station of a digital press similar to the configuration which is described in **EP-A 698 488**. The transfer material can be unwound from said supply roll and the layer containing the dry powder can then be brought in direct contact with the surface of a plate cylinder by one or more contact rollers. After the transfer step, which may be carried out by applying pressure and/or heat on said transfer material while being in contact with the metal support, the used transfer material may be wound up again on a take-up roll. In the latter embodiment, the transfer of dry power can be carried out so as to obtain a uniform layer which then can be image-wise exposed. Alternatively said pressure and/or heat can be applied image-wise, so that the dry powder is transferred image-wise to the metal support. This step then may be followed by intense overall heating, e.g. by infrared laser exposure. However, if sufficient heat is applied during said image-wise transfer, a suitable printing master may directly be obtained without intense overall heating.

In an even more preferred embodiment of the automated method, described above, a dry coating unit as described above, consisting of a supply roll, one or more contact rollers and a take-up roll, is mounted on the same carriage as the laser exposure unit of an external drum image-setter. Reference is made to e.g. Figure 1 of **US-P- 5 713 287** which illustrates a similar device wherein a spray coating unit is mounted on the same carriage as the laser exposure unit in an external drum configuration. In this way, said dry coating unit moves in front of the laser exposure unit along the so-called slow scan axis, parallel to the axis of the plate cylinder. As the plate cylinder is rotated during image-wise exposure (fast scan movement), the whole surface of said cylinder passes the dry coating unit and a layer is coated along a spiral path around the cylinder. Since the laser exposure unit moves together with the dry coating unit, an area which has been coated during one revolution of the cylinder is exposed by the laser exposure unit a number of revolutions later, i.e. coating and image-wise exposing can be carried out almost simultaneously during the same scan procedure.

The materials made according to the present invention can be exposed to light by a light omitting diode or an IR-laser such as an He/Ne or Ar laser. Preferably a laser emitting near infrared light having a wavelength in the range from about 700 to about 1500 nm is used, e.g. a semiconductor laser diode, a Nd:YAG or a Nd:YLF laser. The required laser power depends on the pixel dwell time of the laser beam, which is determined by the spot diameter (typical value of modern plate-setters at 1/e² of maximum intensity : 10-25 µm), the scan speed and the resolution (i.e. the number of distinct pixels per unit of linear distance, often expressed in dots per inch or dpi; typical value : 1000-4000 dpi). A major benefit of the materials made according to the present invention is that they can be used as a universal imaging material which is suitable for exposure by internal (ITD) as well as external drum (XTD) image-setters. ITD image-setters are typically characterised by very high scan speeds up to 500 m/sec and may require a laser power of several Watts. Satisfactory results have also been obtained by using XTD image-setters having a typical laser power from 100 mW to 500 mW at a lower scan speed, e.g. from 0.1 to 10 m/sec.

The materials can even be used as a printing master immediately after image-wise exposure without any additional processing because the unexposed areas are readily removed by the fountain solution or the ink applied during the first runs of the printing job.

The printing plate of the present invention can also be used in the printing process as a seamless sleeve printing plate. In this option the printing plate is soldered in a cylindrical form by means of a laser. This cylindrical printing plate which has as diameter the diameter of the print cylinder is slid on the print cylinder instead of mounting a conventional printing plate. More details on sleeves are given in "Grafisch Nieuws" , 15, 1995, page 4 to 6.

Most printing plates described in the prior art require a so-called post-bake, i.e. an overall heating treatment after image-wise exposure and optional processing so as to increase the run length of the plate. The materials made according to the present invention allow to achieve satisfactory run lengths without a post-bake.

### EXAMPLES

While the present invention will hereinafter be described in connection with preferred embodiments thereof, it will be understood that it is not intended to limit the invention to those embodiments.

### Example 1

An aluminum support was electrochemically roughened using hydrochloric acid , anodized in sulphuric acid and subsequently treated with polyvinylphosphonic acid. The obtained hydrophilic surface was further used for the application of a dry powder.

Dry powders consisting of organic compounds and infrared absorbing compounds were used for rubbing in the above described hydrophilic surface of the electrochemically roughened and anodized aluminum support, using a cotton pad.

Powders with various types and ratios of the organic compound and the IR-absorbing compound were prepared and applied by dry rubbing.

The carbon black containing powders were prepared by mixing the aqueous carbon black dispersion with an aqueous latex or dispersion of the organic compound in an appropriate ratio and freeze drying the aqueous mixture to remove water from the mixture. The carbon black used in these experiments is Printex L6 ™, a trade name of Degussa and the different organic compounds are described in tabel 2.
In the composition 6, the IR-dye was included into the latex particle and in composition 7 the IR-dye was absorbed on the latex particle.

**Table 2**

| Organic compound (particle size) | IR_sensitive compound | Required plane image power | Ratio organic comp./IR-sensitiv comp. |
|---|---|---|---|
| 1.polystyrene(71 nm) | carbon black | between 190 and 292 mW | 90/10 |
| 2.Polystyrene(71nm) | carbon black | ≅190 mW | 55/45 |
| 3.Polymethylmethacrylate(72nm) | carbon black | between 80 and 190 mW | 90/10 |
| 4.Polymethylmethacrylate(72nm) | carbon black | ≅292 mW | 55/45 |
| 5.Novolac(phenol/ cresol resin) | carbon black | <80 mW | 55/45 |
| 6. Polymethylmethacrylate(1µm) | Tab 1 Cpd 7 | between 80 and 190 mW | 94.8/5.2 |
| 7. Polymethylmethacrylate(90nm) | Tab 1 Cpd 7 | >292 mW | 94.8/5.2. |

After rubbing the powder in the hydrophilic aluminum surface, the obtained imaging element was exposed with a 830 nm diode laser (Isomet-3600 dpi (about 1400 dots per cm)-spot size 11 µm-at a speed of 3.2 m/s; i.e. pixel dwell time of 3.4 µs-image plane power was varied :80mW-190mW-292mW were used) and printed on a conventional offset printing machine equipped with a conventional ink and fountain solution.

Printing was started without any treatment between imaging and the press start.

All of the tested compositions resulted in good prints with good image quality.

### Example 2

An aluminum support is electrochemically roughened using hydrochloric acid, anodized in sulphuric acid, and subsequently treated with polyvinylphosphonic acid.

The obtained hydrophilic surface was further used for the application of dry powders consisting of polymethylmethacrylate beads of 1 urn and graphite (Graphite Natural™ trade name of Carbone Lorraine, France- with a particle size < 20 µm as an infrared absorbing compound were used for dry rubbing in the above described hydrophilic surface of an electrochemically roughened and anodized aluminum support, using a cotton pad.

After rubbing the powder in the hydrophilic aluminum surface, the obtained imaging element was exposed with an 830 nm laser diode (Isomet-3600 dpi (about 1400 dots per cm)-spot size 11 µm-at a speed of 3.2 m/s; i.e.pixel dwell time of 3.4 µs-Image plane power was varied: 200 mW and 300 mW were used) as well as with a 1060 nm NdYLF laser (Isomet-3600 dpi (about 1400 dots per cm)-spot size 18 µm-at a speed of 3.2 m/s-image plane power was varied: 585 mW and 780 mW were used) and printed on a conventional offset printing machine equipped with a conventional ink and fountain solution system.

Printing was started without any treatment between imaging and the press start.

All of the tested powders resulted in good image quality, but sensitivity and the lithographic behaviour , e.g. ink-uptake, were different.

The ink-uptake, measured by Dmax on print 100 (see table 3), proves that the organic compound is needed in an amount of at least 51% to print high densities (>1.55 required); without said amount of polymethylmethacrylate-beads high densities print could not be guaranteed.

With only organic compound (no IR-absorbing compound) in the imaging material no image was formed at all.

**Table 3**

| Ratio graphite/polymethylmethacryla te 1µm beads | Dmax (100 sheets) Isomet NdYLF 3.2 m/s | | Dmax (100 sheets) Isomet diode 3.2 m/s | |
|---|---|---|---|---|
| 100/0 | 585 mW | 1.45 | 200 mW | 0.81 |
| | 780 mW | 1.12 | 300 mW | 1.52 |
| 75/25 | 585 mW | 1.41 | 200 mW | 1.42 |
| | 780 mW | 1.52 | 300mW | 1.49 |
| 50/50 | 585mW | 1.43 | 200 mW | 1.51 |
| | 780mW | 1.53 | 300 mW | 1.52 |
| 25/75 | 585mW | 1.61 | 200 mW | 1.55 |
| | 780 mW | 1.61 | 300 mW | 1.60 |

## Claims

1. A method for making a lithographic printing plate comprising the steps of:
(a) making a negative working non-ablative imaging material by applying a dry powder containing at least a compound capable of converting light into heat and an organic compound on a surface of a non-electrically charged metal support, wherein the amount of organic compound in said powder ranges from 51 to 95% by weight;
(b) image-wise exposing the imaging material with an IR-laser;
(c) removing the powder at non-exposed areas by supplying with a printing press fountain solution and/or ink to the imaging material.

2. A method according to claim 1 wherein said organic compound consists of organic thermoplastic polymer particles having a diameter between 0.02 and 10 µm.

3. A method according to claim 1 or 2 wherein said organic compound consists of organic thermoplastic polymer particles having a diameter between 0.05 and 2 µm.

4. A method according to claim 2 or 3 wherein said organic thermoplastic polymer particles have a reactive compound inside or outside said particles.

5. A method according to claim 2 or 3 wherein said organic thermoplastic polymer particles consist of novolac and/or polystyrene and/or a polyacrylate.

6. A method according to claim 1 to 5 wherein the compound capable of converting light into heat is a near infrared absorbing compound.

7. A method according to claim 6 wherein the near infrared absorbing compound is an organic dye or carbon.

8. A method according to claim 6 or 7 wherein the near infrared absorbing compound is heterogeneously mixed with said organic compound.

9. A method according to any of the previous claims wherein the metal support is a sleeve or a cylinder of a rotary printing press.

10. A method according to any of the previous claims wherein between step (b) and step (c) the exposed material is mounted on a printing cylinder of a rotary press.

11. A method according to any of the previous claims wherein between step (a) and step (b) the imaging material is mounted on a printing cylinder of a rotary press.

## Patentansprüche

1. Ein durch die nachstehenden Schritte **gekennzeichnetes** Verfahren zur Herstellung einer lithografischen Druckplatte :
(a) Herstellung eines negativarbeitenden nicht-ablativen Bilderzeugungsmaterials durch Beschichtung einer Oberfläche eines nicht elektrisch geladenen Metallträgers mit einem trockenen Pulver, das zumindest eine Licht in Wärme umwandelnde Verbindung und eine organische Verbindung enthält, wobei die Menge der organischen Verbindung zwischen 51 Gew.-% und 95 Gew.-% liegt,
(b) bildmäßige Belichtung des Bilderzeugungsmaterials mit einem IR-Laser,
(c) Entfernung des Pulvers in den nicht-belichteten Bereichen durch Auftrag von Feuchtwasser und/oder Druckfarbe auf das Bilderzeugungsmaterial.

2. Verfahren nach Anspruch 1, **dadurch gekennzeichnet, dass** die organische Verbindung aus organischen thermoplastischen polymeren Teilchen mit einer Teilchengröße zwischen 0,02 µm und 10 µm besteht.

3. Verfahren nach Anspruch 1 oder 2, **dadurch gekennzeichnet, dass** die organische Verbindung aus organischen thermoplastischen polymeren Teilchen mit einer Teilchengröße zwischen 0,05 µm und 2 µm besteht.

4. Verfahren nach Anspruch 2 oder 3, **dadurch gekennzeichnet, dass** die organischen thermoplastischen polymeren Teilchen innerhalb oder außerhalb der Teilchen eine reaktive Verbindung enthalten.

5. Verfahren nach Anspruch 2 oder 3, **dadurch gekennzeichnet, dass** die organischen thermoplastischen polymeren Teilchen aus Novolak und/oder Polystyrol und/oder einem Polyacrylat bestehen.

6. Verfahren nach einem der Ansprüche 1 bis 5, **dadurch gekennzeichnet, dass** die Licht in Wärme umwandelnde Verbindung eine nahes Infrarotlicht absorbierende Verbindung ist.

7. Verfahren nach Anspruch 6, **dadurch gekennzeichnet, dass** die nahes Infrarotlicht absorbierende Verbindung ein organischer Farbstoff oder Kohlenstoff ist.

8. Verfahren nach Anspruch 6 oder 7, **dadurch gekennzeichnet, dass** die nahes Infrarotlicht absorbierende Verbindung heterogen der organischen Verbindung beigemischt ist.

9. Verfahren nach einem der vorstehenden Ansprüche, **dadurch gekennzeichnet, dass** der Metallträger ein hülsenförmiger Träger oder eine Drucktrommel einer Rotationsdruckpresse ist.

10. Verfahren nach einem der vorstehenden Ansprüche, **dadurch gekennzeichnet, dass** das belichtete Material zwischen Schritt (b) und Schritt (c) auf eine Drucktrommel einer Rotationsdruckpresse aufgespannt wird.

11. Verfahren nach einem der vorstehenden Ansprüche, **dadurch gekennzeichnet, dass** das Bilderzeugungsmaterial zwischen Schritt (a) und Schritt (b) auf eine Drucktrommel einer Rotationsdruckpresse aufgespannt wird.

## Revendications

1. Procédé pour la confection d'une matrice d'impression lithographique comprenant les étapes consistant à :
- préparer un matériau de formation d'image non ablative à effet négatif en appliquant une poudre sèche, contenant au moins un composé capable de transformer de la lumière en chaleur ainsi qu'un composé organique, sur la surface d'un support métallique exempt de charge électrique, la quantité du composé organique dans ladite poudre variant entre 51 et 95% en poids ;
- exposer ledit matériau de formation d'images à l'aide d'un laser infrarouge ;
- éliminer la poudre dans les zones de non-impression en amenant une solution de mouillage et/ou de l'encre au matériau de formation d'image à l'aide d'une presse d'impression.

2. Procédé selon la revendication 1, **caractérisé en ce que** ledit composé organique se compose de particules polymères thermoplastiques organiques possédant un diamètre entre 0,02 et 10 *µ*m.

3. Procédé selon la revendication 1 ou 2, **caractérisé en ce que** ledit composé organique se compose de particules polymères thermoplastiques organiques possédant un diamètre entre 0,05 et 2 *µ*m.

4. Procédé selon la revendication 2 ou 3, **caractérisé en ce que** lesdites particules polymères thermoplastiques organiques possèdent un composé réactif à l'intérieur ou à l'extérieur desdites particules.

5. Procédé selon la revendication 2 ou 3, **caractérisé en ce que** lesdites particules polymères thermoplastiques organiques se composent de novolaque et/ou de polystyrène et/ou d'un polyacrylate.

6. Procédé selon les revendications 1 à 5, **caractérisé en ce que** ledit composé capable de transformer de la lumière en chaleur est un composé absorbant la lumière dans le domaine de l'infrarouge proche.

7. Procédé selon la revendication 6, **caractérisé en ce que** ledit composé absorbant la lumière dans le domaine de l'infrarouge proche est un colorant organique ou le carbone.

8. Procédé selon la revendication 6 ou 7, **caractérisé en ce que** ledit composé absorbant la lumière dans le domaine de l'infrarouge proche est mélangé d'une manière hétérogène avec ledit composé organique.

9. Procédé selon l'une quelconque des revendications précédentes, **caractérisé en ce que** ledit support métallique est un manchon ou un cylindre d'une presse rotative.

10. Procédé selon l'une quelconque des revendications précédentes, **caractérisé en ce que** le matériau exposé est monté sur un cylindre d'impression d'une presse rotative entre l'étape (b) et l'étape (c).

11. Procédé selon l'une quelconque des revendications précédentes, **caractérisé en ce que** le matériau de formation d'image est monté sur un cylindre d'impression d'une presse rotative entre l'étape (a) et l'étape (b).
